

Patented July 25, 1933

1,919,526

# UNITED STATES PATENT OFFICE

OSKAR OPPENLAENDER, OF ELIZABETHTON, AND RICHARD ELSSNER, OF JOHNSON CITY, TENNESSEE, ASSIGNEES TO AMERICAN GLANZSTOFF CORPORATION, OF NEW YORK, N. Y., A CORPORATION OF DELAWARE

## UNTWISTED DIRECT PROCESS YARN WITH EVEN SHRINKAGE

No Drawing.

Application filed July 2, 1932. Serial No. 620,724.

In the treatment of artificial silk, such as the process disclosed in copending application Serial Number 548,474 (applicants Bitter and Elssner), a procedure which may be followed in order to produce an even shrinkage of the yarn, is set forth. In application 548,474, the filaments are covered with an impermeable covering, and are dried from one side only. In this way the drying medium acts from one side only (the inner side) of the yarn body, and all the moisture in the spool is taken from the said inner side. Usually, it is necessary that filaments so dried be rewound, and, after rewetting, redried in the same way.

The present invention, however, concerns a new method wherein the yarn body may be caused to produce an even shrinkage by a single drying only.

As is well known, when filaments are dried in the ordinary manner, on perforated spools, the heated air is applied to both the surfaces, the outer layers immediately dry, while the central layers are heated so that a very humid condition is produced there. This results in the formation of an unyielding mass of moist or wet layers of thread which prevents the outer layers of the yarn body from shrinking. The inner layers, similarly, are pressing against the central portion of the spool which is likewise an unyielding surface and accordingly, dry without proper shrinkage. The central layers, however, do shrink. The resulting yarn body has a total uneven shrinkage which affects its physical properties and the manner in which it will take dyes.

In the present process, however, the yarn is directly collected, on extrusion, upon so-called collapsible spools. This term is to be construed to mean a spool, the surface of which is slotted, wherein wings or fins are caused to project through the slots during the winding of the filaments. These fins or wings cause the surface of the spool to be incremented in size during the time that the filaments are being wound thereon. When the winding is completed the fins or blades are allowed to retract, and the wound yarn body thereupon lies loosely upon the spool body per se.

In the present process, filaments are so wound, and then allowed to lie loosely on the body of the spool by decreasing the winding surface in the manner set forth. After treatment of the filaments is necessary since they

must be deacidified, desulphurized, etc. These steps take place on the spool, and while still wet, the outer surface of the spool is covered with an impermeable covering. The drying medium, for example, air, is then applied to the filaments from the inside only. Drying, accordingly, occurs from one side only.

It may thus be seen that, in a single drying, a yarn with even shrinkage may be produced. In the old method of drying from all sides at once, on rigid spools, as pointed out above, the outer and innermost filaments of the body do not have an opportunity to contract or shrink. In the present process, the innermost filaments dry first. Because they are in a relaxed state and are loosely lying upon the spool core, they are given an opportunity to shrink properly. The central portion and outermost portions, meanwhile, are being slowly dried. As each successive layer of the filament body dries, it has ample opportunity to contract or shrink, and, therefore, when the outermost layers have finally dried, a yarn body with even shrinkage is produced.

It is not an object of the present invention to attempt to cover the construction of any collapsible spool, but what is claimed is:

1. In a process for treating artificial filaments, threads, etc., the steps of collecting them upon a spool or bobbin, retracting the winding surface so that the filaments etc. lie in a loose body upon the spool or bobbin, wet-treating the filaments, etc., covering the outer surface thereof with an impermeable covering, and then drying the yarn body from the inside of the spool or bobbin only.

2. In a process of producing artificial filaments or yarn with an even shrinkage, the steps of winding the yarn on a spool the winding surface of which may be lessened in periphery, and, after reducing the said surface so that the yarn body lies loosely thereon, washing and drying the filaments, the drying step being accomplished by covering the outer surface of the yarn body and drying from the inner side only.

OSKAR OPPENLAENDER.  
RICHARD ELSSNER.

105

110